

1

2,715,106

**LUBRICATING OIL COMPOSITION**

Elmer W. Brennan, Carpentersville, Ill., and Harold G. Raybould, Jr., Tulsa, Okla., assignors to The Pure Oil Company, Chicago, Ill., a corporation of Ohio

No Drawing. Application December 29, 1951,  
Serial No. 264,275

5 Claims. (Cl. 252—33.4)

This invention relates to a lubricating oil composition having increased performance characteristics. It is more specifically concerned with enhancing the antiweld properties of lubricating oil blends.

In the development of improved lubricating oils, rather than relying exclusively on physical and chemical refining methods to produce a desirable product, lubricating manufacturers have resorted to the use of various chemical compositions which when added to a mineral oil base impart desirable properties to the oil. While in some instances the additives are employed to obviate the use of expensive operations another important use for additives is to provide the mineral oil base with lubricating qualities not inherently possessed by mineral oils. One of the most important deficiencies of mineral oils is the inability to provide lubrication between moving parts which develop during their operation contact pressures which are extremely high. In order that mineral oil lubricants may be used as gear lubricants it is vital that suitable extreme pressure adducts be admixed with the mineral oil. A multitude of types of compounds have been suggested in the prior art for this purpose. Various compositions containing lead, sulfur, chlorine or phosphorus substituents or combinations of these substituents have found wide use in this application. For determining the efficacy of specific compounds a wide variety of gear lubricant testing procedures have been developed. These tests include both field service tests where actual performance is evaluated under actual operating conditions using automotive vehicles and laboratory tests in which full scale axle assemblies or laboratory bench test machines are used. In employing laboratory facilities to test gear lubricants, bench tests are used generally to predict the service performance of gear lubricants. Some of the more widely used machines which incorporate the action of one metal surface sliding on another are the Almen, Falex, 4-Ball, SAE and Timken. In demonstrating the instant invention a Falex machine was employed to provide test data. In the Falex machine, test pieces consist of a  $\frac{1}{4}$  inch diameter steel journal and two V-blocks. The steel journal is held in a vertical shaft by means of a brass shear pin. This journal is caused to rotate at a constant speed. Two lever loading arms separately pivoted behind the vertical spindle have self-aligning recesses in them to take the V-blocks. The blocks are assembled in place in such a manner that the V notches are vertical and clamped around the steel journal, being so mounted as to permit torque measurement. A load is applied by means of a suitable mechanism which by means of a large ratchet wheel on rotation increases the load by squeezing the two lever loading arms together. The load applied is registered on a loading dial which records the actual load applied to the V-blocks. The machine may be adjusted

2

so that the ratchet wheel will be turned automatically thus applying the load at a standard rate. It may also be turned manually if desired. The torque set up by the journal rotating against the V-blocks is indicated by a hydraulically operated pressure gauge, the V-shaped bearing blocks and entire load applying mechanism being free to turn about the axis of the test journal. In evaluating a gear oil lubricant, a sample of the oil is placed in a metal oil cup and the two V-blocks and journal are immersed in the oil.

Many different test procedures have been suggested for use with this machine. In evaluating the lubricating composition employed in the instant invention two tests were used, namely, the hour wear test and the maximum load test. In the former test the machine was operated under conditions whereby a constant load was applied to the test blocks. The number of teeth wear on the ratchet wheel indicate whether or not the oil under test was satisfactory. In evaluating a lubricating oil composition by means of the maximum wear test the ratchet wheel is automatically turned thereby applying incremental increases in load to the V-blocks at a standard rate. This test may be accompanied by scoring of the test surfaces or shearing of the journal or shear pin. In this instance the maximum load which the oil is capable of withstanding is used as a criterion of performance characteristics.

As it has been pointed out various types of compounds have been used as extreme pressure lubricating oil additives. Included among the available and applicable compounds are the terpene hydrocarbons or their derivatives which when sulfurized and phosphorized produce a composition which if added to a mineral oil base would serve to increase the anti-weld properties of a mineral oil. While these materials function effectively as anti-wear additives, there is an optimum amount that can be added to the mineral oil composition beyond which the small increase in effect obtained does not justify the addition of larger amounts.

It is therefore the object of this invention to enhance the anti-weld properties of mineral oil gear lubricants by adding to a lubricating oil composition containing minor proportions of sulfurized and phosphorized terpenes minor amounts of an additional beneficiating agent to the lube oil composition thereby unexpectedly increasing the anti-weld properties thereof. This and other objects of the invention will become apparent from the following description of this invention:

In accordance with this invention it has been found that the anti-weld properties of a sulfurized and phosphorized terpene-containing lubricating composition are synergistically improved by the addition of minor amounts of an alkali metal oil soluble organic sulfonate. Although the use of sulfonates as extreme pressure agents is disclosed in the prior art, sulfonates generally are employed as wetting agents in lubricating oil compositions and under these conditions do not impart an unexpected increase in the extreme pressure properties of mineral oil blends containing them. However, when these sulfonates are present in an amount between 0.5 and 5 per cent by weight and preferably about 1 per cent by weight in a sulfurized and phosphorized terpene-containing mineral oil lubricant, an unexpected increase in the anti-weld properties of the composition is obtained. To illustrate the instant invention Falex test data were obtained on blends of mineral oil and varying concentrations of sodium petroleum sulfonate, mineral oil blends containing a sulfurized and phosphorized terpene alcohol and mineral oil blends containing sulfonates and a sulfurized and phosphorized terpene.

phorized terpene alcohol. These results are shown in Table I.

TABLE I  
*Falex test data*

| Composition                             | Hour Wear    |              | Max. Load |
|-----------------------------------------|--------------|--------------|-----------|
|                                         | Load, Pounds | Tooth Wear   |           |
| 8.5% Sulfo-phosphorized terpene alcohol |              |              |           |
| 91.5% mineral oil base                  | 800          | 147-----     | 2,500     |
| 8.5% sulfo-phosphorized terpene alcohol | 800          | 80-----      |           |
| 0.5% alkali metal petroleum sulfonate   |              |              |           |
| 91.0% mineral oil base                  |              |              |           |
| 8.5% sulfo-phosphorized terpene alcohol | 800          | 33-----      | 2,250     |
| 1.0% alkali metal petroleum sulfonate   | 400          | seizure----- | 900       |
| 99.5% mineral oil base                  | 800          | do-----      |           |
| 1.0% alkali metal petroleum sulfonate   | 400          | 30-----      | 1,200     |
| 99.0% mineral oil base                  | 800          | seizure----- |           |
| 1.5% alkali metal petroleum sulfonate   | 400          | do-----      | 900       |
| 98.5% mineral oil base                  | 800          | do-----      |           |
| 10% alkali metal petroleum sulfonate    | 400          | 32-----      | 900       |
| 90% mineral oil base                    | 800          | seizure----- |           |
| 100% mineral oil base                   | 400          | do-----      | 900       |

The test results shown in Table I demonstrate the effective action of combinations of a sulfurized and phosphorized terpene and minor amounts of an alkali metal oil soluble organic sulfonate admixed in a mineral oil base. It is seen that the mineral oil composition containing sodium petroleum sulfonate in concentrations as high as 10% failed in the Falex hour wear test when evaluated with an 800 lb. load. This indicates that the sulfonates alone under these conditions do not impart to the mineral oil base any extreme pressure characteristics. However, mineral oil compositions containing only a sulfurized and phosphorized terpene do function as extreme pressure additives. However, the use of an oil soluble alkali metal organic sulfonate in combination with a sulfurized and phosphorized terpene improves the wear characteristics of the mineral oil composition with little deleterious results upon the maximum load results obtained, a phenomenon which could not be predicted from the test results obtained when using each of the blend components alone in combination with a mineral oil base. It is thus seen that superior performance characteristics relative to the extreme pressure properties of a lubricating oil are provided when minor proportions of a sulfurized and phosphorized terpene and an oil soluble alkali metal organic sulfonate are admixed in a mineral oil base.

The sulfurized and phosphorized terpene alcohol employed in illustrating the instant invention was prepared by slowly heating one mole of a bicyclic terpene alcohol, methylol beta pinene, having a formula  $C_{11}H_{17}OH$ , to a temperature of approximately 270° F. An equimolar proportion of pulverulent sulfur was sifted into the heated terpene. After the addition of sulfur the temperature was raised to approximately 330° F. and maintained at substantially this temperature until a satisfactory copper strip corrosion test was obtained. In this instance about eight hours was required during which period the mixture was continuously agitated. The mixture was then allowed to cool to a temperature of about 180° F. About 0.4% by weight of finely divided phosphorus sesquisulfide was admixed with the sulfurized base and heat applied to the mixture while it was continuously agitated. The temperature was raised to about 220° F. and maintained at about this temperature until the reaction was completed, about five hours being sufficient under these conditions. The mixture was then allowed to cool. The finished product was a composition containing 15.7 weight per

cent sulfur, and 0.22 weight per cent phosphorus and having a viscosity of 281 S. U. S. at 210° F.

Although the sulfurization and phosphorization of a terpene alcohol is above described it will be understood that other substituted or unsubstituted isoprenoids may be employed. For example, camphene, dipentene, pinene, terpineol, isopulegol may be used. Similarly, reasonable latitude may be employed in selecting the other reagents as well as the amounts used. In preparing the sulfurized-phosphorized additive the amount of sulfur may vary within wide limits, depending upon the terpene being treated. For example, in sulfurizing dipentene a sulfurized product containing about 30% by weight of sulfur can be obtained. In carrying out the initial sulfurization reaction substantially stoichiometric amounts of sulfur are employed and the sulfurization reaction is carried to substantial completion as evidenced by a negative copper strip test. Any excessive amounts of unused reactants are separated from the finished product. However, the sulfur content of the chemically treated terpene should be sufficient to provide the mineral oil composition containing the sulfurized and phosphorized terpene with an added sulfur content attributable to the presence of the said terpene of between about 0.2 and 1.8% by weight and preferably about 1.25% by weight. Phosphorus compounds such as the oxides, halides, or other sulfides may be used as alternatives in place of the sesquisulfide. The amount of phosphorus in the sulfurized and phosphorized product should not exceed 2 per cent and preferably should be only a fraction of 1 per cent, preferably 0.2 to 0.6 per cent based on the weight of sulfurized base.

The sulfonates which are admixed in the mineral oil base in combination with the sulfurized and phosphorized terpene may be any oil soluble alkali metal salt of sulfonic acid. The alkali metal petroleum sulfonates however are preferred.

What is claimed is:

1. A lubricating composition comprising a mineral oil base having admixed therein minor proportions of a sulfurized-phosphorized terpene alcohol in an amount sufficient to impart anti-wear characteristics to said mineral oil and an oil soluble alkali metal organic sulfonate in an amount sufficient to enhance the effectiveness of said alcohol as an anti-wear agent.
2. A composition in accordance with claim 1 in which said sulfonate is a sodium petroleum sulfonate.
3. A mineral oil lubricating composition having enhanced anti-wear properties which contains an amount of a sulfurized and phosphorized terpene alcohol sufficient to provide said composition with an added sulfur content attributable to said terpene of between about 0.2 to 1.8 per cent by weight, and about 0.5 to 5 per cent by weight based on total composition of an oil soluble alkali metal organic sulfonate.
4. A composition in accordance with claim 3 in which about 1 per cent by weight of said sulfonate is present.
5. A lubricating composition which comprises a mineral oil containing about 8.5 per cent by weight of a phosphorized and sulfurized methylol beta pinene and 1 per cent by weight of a sodium petroleum sulfonate based on total composition, said sulfurized-phosphorized pinene containing about 16 per cent by weight of sulfur and about 0.2 to 0.25 per cent by weight of phosphorus based on said pinene.

65  
References Cited in the file of this patent  
UNITED STATES PATENTS

2,379,453 Noland ----- July 3, 1945  
2,416,281 Berger et al. ----- Feb. 25, 1947